

Patented Jan. 26, 1926.

1,570,802

# UNITED STATES PATENT OFFICE.

FOORD VON BICHOWSKY, OF GLENDALE, CALIFORNIA.

## MEANS FOR PREVENTING ADHERENCE OF CAST METAL TO THE MOLD.

No Drawing.

Application filed April 22, 1924. Serial No. 708,312.

To all whom it may concern:

Be it known that I, FOORD VON BICHOWSKY, a citizen of the United States, and a resident of Glendale, county of Los Angeles, State of California, have invented a new and useful Means for Preventing Adherence of Cast Metal to the Mold, of which the following is a specification.

This invention relates to the formation 10 of an inert layer of material upon the surface of the mold whereby adherence of the cast metal to the mold is prevented and consequently castings of much higher quality and appearance may be produced.

15 In this making of casting, particularly from steel and high melting point alloys, much trouble has been encountered for the temperature at which these melts are poured into the mold lies so close to the melting 20 point of the molding sand that considerable of the silica attaches itself firmly to the casting and therefore expensive grinding and sand blasting are required before the casting can be machined.

25 In order to minimize this adherence, or burning in, of the molding sand to the casting it is the practice for the molder to dust the finished mold over with silica flour, i. e. very fine molding sand, with a view of obtaining a smoother mold surface so that the molten metal will be less apt to adhere. It is also the practice to coat the inside of the mold with a thin skin of carbon, deposited 30 from a smoky acetylene flame but in many cases this cannot be done as the molten metal may absorb the carbon to form a brittle surface skin or a lower melting point alloy. This reason likewise prevents the 35 use of graphite.

40 The number of materials that might be used to prevent sticking of the metal to the mold by being interposed in the form of a thin skin over the surface of the mold is limited. For first of all such material must 45 remain unaltered as the temperature of the molten metal or at least until the metal has solidified. Second, the material must be chemically neutral to both the molding sand and to the metal being cast, otherwise 50 an impervious film would be formed so that the mold gases could not escape and the casting would then either be completely ruined or else would contain numerous gas cavities. The free venting of the mold, 55 and especially the core, is most essential in casting electric steels and the other elec-

tric furnace alloys. As a final quality the protective material must be of such a nature as to make it easy of removal from the finished casting.

60 In searching about for such an ideal material I have experimented with certain nitrides and have discovered that they are most suitable for this purpose. This is especially true of the nitrides of silicon, 65 titanium, aluminium, boron and zirconium. These are all quite stable bodies decomposed by heat only at extremely high temperature, and but slowly attacked by the oxygen of the air. Because of these valuable properties it has already been proposed to employ these nitrides, in the form of molded blocks for the lining of electric furnaces, Serpek United States Patent No. 1,099,131, and of crucibles, Podszus German Patents 75 Nos. 282,748 and 286,992. Employed in this manner the density of the blocks would naturally confine any destructive action to the outside surfaces and consequently their life 80 would be prolonged.

I began to experiment with the nitrides of titanium and the mixed aluminium and silicon nitrides. But as I proposed to use them in the form of powder there was no certainty that they would stand up or 85 would not unite with the molten steel. In the first experiment I dusted these materials, in the form of a very fine powder, on the surface of the mold but the results were not very satisfactory as the flowing molten steel 90 tended to wash them away and then to combine with the sand thereby exposed. This action can be greatly reduced by using the nitrides in a coarser form. However, when these nitrides were mixed to the consistency 95 of paint, with water, and then sprayed or bushed on the mold excellent results were obtained and this was especially noticeable with the cores.

100 Continuing the experiments I discovered that it was not necessary to use pure nitrides but that the crude nitride produced under the methods of United States Patents Nos. 1,391,147, 1,391,148, 1,408,661 and 1,415,280 and which often contained almost half their 105 weight of finely divided iron could be used with equally satisfactory results if made into a thin wash with water, either pure or else containing a small quantity of binding material such as molasses, sodium silicate, salt or other suitable agent or agents; or sprayed or painted on the mold and core 110

which were then dried either by "skin-drying" with an open flame or by other means. If necessary the above spraying and drying procedure may be repeated one or more times in order to obtain a sufficiently thick coat. This treatment gives to the mold a smooth surface which remains porous to the mold gases at all temperatures. Upon removing the casting from a mold so treated a simple sand blasting is all that is necessary before the casting is ready for machining. It is surprising that these crude nitrides with so much iron should be so resistant but this is due no doubt to the extremely fine state of division of that element so that no considerable surface is presented either to the sand or to the molten alloy, and besides this the iron probably plays a part in that it allows a uniform rate of heat exchange between the hot iron and the cool mold and so prevents an unequal chilling of the surface metal. In using these nitrides in the form of a wash it is necessary that they be finely ground and that the vehicle in which they are suspended be kept stirred or in constant agitation.

For the purpose of our claims the term mold is used to define both the form and the cores whether constructed of sand or of any

other material such as iron or steel (billet 30 molds) clay, etc. Under the term nitrides I include the so-called carbo-nitride or cyanonitrides.

Having now described my invention and the method of carrying it into effect what I 35 claim is:

1. A coating compound for molds of the character described comprising a substance containing an appreciable quantity of combined nitrogen in the form of a nitride of 40 a member of the carbon group of elements.

2. A coating compound for molds of the character described comprising a substance containing an appreciable quantity of combined nitrogen in the form of a nitride of 45 titanium.

3. A coating compound for molds of the character described comprising a substance containing an appreciable quantity of combined nitrogen in the form of crude titanium 50 nitride associated with metallic iron.

4. A coating compound for molds of the character described comprising a substance containing an appreciable quantity of combined nitrogen in the form of a nitride of a 55 member of the carbon group of elements and associated with metallic iron.

FOORD VON BICHOWSKY.